

## 1

3,535,212

## NICKEL PLATING PROCESS

Slavko M. Dobrash, Warren, and William R. Vincent,  
Birmingham, Mich., assignors to General Motors Corporation, Detroit, Mich., a corporation of Delaware  
No Drawing. Filed July 6, 1966, Ser. No. 563,053  
Int. Cl. C23b 5/50

U.S. CL. 204—29

6 Claims

## ABSTRACT OF THE DISCLOSURE

A preplating treatment for nickel plating onto zinc in which the zinc is first coated with a film of an alkyl or an alkanolamine prior to immersion into the nickel plating bath.

This invention relates generally to the nickel plating of zinc and, more specifically, to a preplating treatment for use prior to the actual plating sequence.

The pre-plating treatment of our invention is most significantly effective when used prior to practicing the nickel plating process disclosed and claimed in copending U.S. patent application Ser. No. 516,761, Baig, filed Dec. 27, 1965 now U.S. Pat. No. 3,417,005. However, the process disclosed and claimed herein is applicable to other nickel plating processes too. The previously mentioned Baig patent application is directed toward a nickel electrodeposition bath and the process for its use. The bath disclosed and claimed therein, briefly described, comprises:

At least 0.53 mole/liter of nickel ion ( $Ni^{++}$ ); at least 0.45 but less than 0.54 mole/liter of citrate ion ( $C_6H_5O_7^{---}$ ); at least 0.023 mole/liter of gluconate ion ( $C_6H_{11}O_7^{---}$ ); an ion from the group consisting of  $Cl^-$  and  $F^-$  for inducing anode corrosion; and, an additive from the group consisting of  $(NH_4^+)$  and (triethanolamine) for relieving stresses in the deposit.

More specifically, the Baig bath comprises:

| Ions                               | Grams per liter | Moles per liter |
|------------------------------------|-----------------|-----------------|
| Nickel ( $Ni^{++}$ )               | 31-62           | 0.53-1.06       |
| Citrate ( $C_6H_5O_7^{---}$ )      | 85-103          | 0.45-0.54       |
| Gluconate ( $C_6H_{11}O_7^{---}$ ) | 4.5-40          | 0.023-0.21      |
| Chloride ( $Cl^-$ )                | 1-24            | 0.028-0.68      |
| Ammonium ( $NH_4^+$ )              | 1-24            | 0.055-1.33      |

NOTE.— $(H^+)$  or  $(OH^-)$  to adjust pH to 5.0-9.5.

Briefly described, the process disclosed and claimed in the aforementioned Baig application comprises the steps of cleaning the part to be plated; immersing the part into a bath comprising the aforementioned constituents; applying a voltage such as to effect a current density from about 10-150 amps/ft.<sup>2</sup>; removing the part from the bath and rinsing it.

The aforementioned bath and process effectively produces adherent nickel deposits on a variety of metals, including zinc. However, we have found that the deposit will adhere to zinc significantly better if the zinc is pretreated immediately prior to its immersion into the plating bath. By zinc, we mean to include not only the pure metal, but also alloys thereof having a zinc content in excess of 50% by weight.

It is, therefore, an object of our invention to effect a more strongly adherent nickel deposit on zinc substrates.

It is a further object of our invention to improve the process for the electrodeposition of strongly adherent nickel deposits on zinc substrates, which process is described and claimed in U.S. patent application Ser. No. 516,761, Baig, filed Dec. 27, 1965 now U.S. Pat. No. 3,417,005.

These and other objects of our invention will become apparent from the detailed description which follows.

## 2

Briefly stated, our invention comprises immersing a zinc article into a nickel complexing film-forming alkyl or alkanol amine immediately prior to the immersion of the article into the nickel plating bath. By nickel complexing film-forming alkyl or alkanol amine, we mean to include such compounds as the methyl, ethyl, and propyl amines, the methanol, ethanol, and propanol amines, and the ethylene and propylene diamines and derivatives thereof, such as ethylene diamine tetracetic acid. Aqueous solutions of triethanolamine have been found to be significantly effective. In our preferred process for nickel plating zinc base die castings, we immerse them for 15-30 seconds in a 2-10% by volume solution of triethanolamine and then electroplate them with the bath disclosed as preferred for zinc base die castings in the aforementioned Baig patent application. This preferred Baig bath as disclosed in the aforementioned copending application comprises:

| 20                          | Salts   | Grams per liter | Moles per liter |
|-----------------------------|---------|-----------------|-----------------|
| $NiSO_4 \cdot 6H_2O$        | 140-280 | 0.53-1.06       |                 |
| $Na_2C_6H_5O_7 \cdot 2H_2O$ | 132-155 | 0.45-0.53       |                 |
| $Na_2C_6H_{11}O_7$          | 10-30   | 0.046-0.14      |                 |
| $Cl^-$                      | 8-12    | 0.23-0.34       |                 |
| $NH_4^+$                    | 8-12    | 0.44-0.68       |                 |

25 NOTE.—pH, 6.7-7.5. Temperature, 130°-150° F.

Any nickel salt can be used as a source of nickel ions, such as nickel chloride, nickel fluoborate, nickel sulfonate, or nickel acetate. However, the best results have 30 been obtained using nickel sulfate, commercially available in the 6-hydrate or 7-hydrate form.

Concentrations of less than 2% by volume of triethanolamine improve the adhesion of nickel to zinc, which has been treated therewith. However, the improvement in 35 adhesion does not become significant until concentrations in excess of 2% are employed. Concentrations in excess of 10% are effective, but not necessary, and in some respects may even be undesirable, as will be discussed hereinafter in conjunction with the undesirable effects incident to drag-out from the pretreatment bath.

The following is a preferred process that is intended merely to serve as a specific example of our invention for producing an improved, more strongly adherent electrodeposited nickel coating on zinc. An unbuffed zinc die

40 casting such as a door handle was cleaned anodically at a current density of about 50 a.s.f. by immersion into a commercial alkaline cleaner, such as Northwest #371, and was treated therein for about one minute at about 150° F. The part was subsequently rinsed in water followed by a 10 second dip at room temperature in a 4 oz./gal. aqueous solution of an acid salt, such as Northwest 45 Actisalt #1, and a wetting agent, such as Northwest Addition Agent #9. The acid dip was followed by a water rinse. The part was next dipped for about 30 seconds in 50 a 100 ml./gal. (2.6% by volume) aqueous solution of triethanolamine at room temperature. Immediately, without rinsing, the thus treated part was immersed live into 55 a bath comprising:

| 60                 | Ions  | G./l. |
|--------------------|-------|-------|
| $Nickel sulfate$   | 142.2 |       |
| $Nickel chloride$  | 29.92 |       |
| $Sodium citrate$   | 140   |       |
| $Sodium gluconate$ | 29.92 |       |
| $Ammonium sulfate$ | 33.9  |       |

65 The bath had a pH of 7.0 and was maintained at a temperature of about 140° F. Live entry at a strike current density of 150 a.s.f. for about 30 seconds followed by a normal plating current density of 40 a.s.f. for 14 minutes produced optimum coverage and adhesion. A dual chrome 70 layer was then applied in the normal and accepted manner. However, the post nickel plating steps chosen are

wholly dependent upon the nature of the article sought to be produced and may comprise any of the conventional plating sequences known in the art.

We prefer to use the lowest concentration of amine which will produce the desired nickel complexing film. This is preferred in order to prevent any substantial drag-out and incident buildup of amine in the nickel plating bath. Hence, for example, the Baig bath has a limited tolerance for triethanolamine as disclosed in the aforementioned application. Too high a triethanolamine concentration in the bath tends to produce a cracked deposit. Hence, by reducing the concentration of the amine, e.g., triethanolamine, in the preplating treatment step, continuous plating may be effected for a longer period of time before the nickel plating bath must be decontaminated or replaced. As the plating baths vary, so also will their respective tolerances for amines. Hence, the particular plating bath selected from the many known in the art will, in many respects, dictate not only the particular choice of amines, but also the optimum concentration for its use with that particular bath.

The treatment of our invention forms a film over the surface of the article. Exactly what function this film performs is not known. One possible explanation is that the film insulates the surface from oxidation during its traverse from the pretreatment tank to the plating tank and that the film is destroyed upon entry into the plating tank. Another possible explanation may reside in the fact that only compounds which are known to complex nickel seem to be effective and that it is the ability to complex that produces the improved result. We do not intend, however, to be bound by either of these theories.

While we have disclosed our invention in conjunction with a specific embodiment, we do not intend to limit ourselves, except as by recited in the claims appended hereto.

We claim:

1. A process for nickel plating zinc articles comprising the successive steps of immersing a zinc article into a nickel complexing agent consisting essentially of an aqueous solution containing at least about 2% of a compound selected from the group consisting of alkylamines and alkanol-amines, and thereby forming a film of said nickel complexing agent on the surface of said zinc article; immediately subsequently immersing said zinc article already coated with said film of nickel complexing agent into a nickel salt solution; and electrodepositing a strongly ad-

herent nickel coating from the nickel salt solution onto the surface of the zinc article.

2. A process as described in claim 1 wherein said selected compound is triethanolamine.

3. A process as described in claim 2 wherein said nickel salt solution has a pH of about 5.0-9.5 and comprises: (a) a nickel ion concentration of at least 0.53 moles/liter produced from salts selected from the group consisting of nickel sulfate, nickel chloride, nickel fluoborate, nickel sulfonate, and nickel acetate, (b) a citrate ion concentration of at least 0.45 but less than 0.54 mole/liter of solution, (c) a gluconate ion concentration of at least about 0.023 mole/liter of solution, (d) an ion for inducing anode corrosion selected from the group consisting of chloride and fluoride, and (e) an additive for reducing stress in the deposit selected from the group consisting of ammonium ions and triethanolamine.

4. The process as claimed in claim 1 wherein the concentration of said nickel complexing compound is about 2-10% by volume, the balance being water.

5. The process as claimed in claim 4 wherein said complexing compound is triethanolamine.

6. The process as claimed in claim 5 wherein the nickel salt solution has a pH of about 5.0-9.5 and comprises: (a) a nickel ion concentration of at least 0.53 mole/liter produced from salts selected from the group consisting of nickel sulfate, nickel chloride, nickel fluoborate, nickel sulfonate and nickel acetate, (b) a citrate ion concentration of at least 0.45, but less than 0.54 mole/liter of solution, (c) a gluconate ion concentration of at least about 0.023 mole/liter of solution, (d) at least one ion for inducing anode corrosion selected from the group consisting of chloride and fluoride, and (e) an additive for reducing stress on the deposit selected from the group consisting of ammonium ions and triethanolamine.

#### References Cited

##### UNITED STATES PATENTS

|           |         |         |       |        |
|-----------|---------|---------|-------|--------|
| 2,355,070 | 8/1944  | Harford | ----- | 204—49 |
| 3,082,156 | 3/1963  | Brown   | ----- | 204—49 |
| 3,417,005 | 12/1968 | Baig    | ----- | 204—32 |

WINSTON A. DOUGLAS, Primary Examiner

O. F. CRUTCHFIELD, Assistant Examiner

U.S. CL. X.R.

204—32, 49